



US007910278B2

(12) **United States Patent**  
**Ohta et al.**

(10) **Patent No.:** **US 7,910,278 B2**  
(45) **Date of Patent:** **Mar. 22, 2011**

(54) **TONER FOR DEVELOPING  
ELECTROSTATIC IMAGE**

(75) Inventors: **Gen-ichi Ohta**, Tokyo (JP); **Hiroto Kidokoro**, Tokyo (JP)

(73) Assignee: **Zeon Corporation**, Tokyo (JP)

(\*) Notice: Subject to any disclaimer, the term of this patent is extended or adjusted under 35 U.S.C. 154(b) by 943 days.

(21) Appl. No.: **11/793,658**

(22) PCT Filed: **Dec. 28, 2005**

(86) PCT No.: **PCT/JP2005/024071**

§ 371 (c)(1),  
(2), (4) Date: **Jun. 21, 2007**

(87) PCT Pub. No.: **WO2006/070870**

PCT Pub. Date: **Jul. 6, 2006**

(65) **Prior Publication Data**

US 2007/0269733 A1 Nov. 22, 2007

(30) **Foreign Application Priority Data**

Dec. 28, 2004 (JP) ..... 2004-382119

(51) **Int. Cl.**  
**G03G 9/00** (2006.01)

(52) **U.S. Cl.** ..... **430/111.41; 430/125.3**

(58) **Field of Classification Search** ..... **430/111.41,  
430/125.3**

See application file for complete search history.

(56) **References Cited**

**U.S. PATENT DOCUMENTS**

6,613,490 B2 \* 9/2003 Matsunaga et al. .... 430/109.3  
7,026,086 B2 \* 4/2006 Kashiwabara et al. .... 430/108.4  
2003/0044708 A1 \* 3/2003 Matsunaga et al. .... 430/108.22

**FOREIGN PATENT DOCUMENTS**

|    |               |         |
|----|---------------|---------|
| JP | 5-100477      | 4/1993  |
| JP | 9-106093      | 4/1997  |
| JP | 10-171156     | 6/1998  |
| JP | 2000-131877 A | 5/2000  |
| JP | 2001-075305 A | 3/2001  |
| JP | 2001-305779   | 11/2001 |
| JP | 2004-151638   | 5/2004  |
| JP | 2004-198692   | 7/2004  |

**OTHER PUBLICATIONS**

Japanese Office Action dated Sep. 21, 2010, issued in corresponding Japanese Patent Application No. 2006-550845.

\* cited by examiner

*Primary Examiner* — Mark A Chapman

(74) *Attorney, Agent, or Firm* — Westerman, Hattori, Daniels & Adrian, LLP

(57) **ABSTRACT**

The present invention provides a toner for developing electrostatic image comprising a colored particle containing a binder resin, a colorant and a release agent, wherein the toner for developing electrostatic image has two or more peaks of loss tangent ( $\tan \delta$ ) in the range from 50 to 120° C., a loss tangent ( $\tan \delta$ ) in the range from 100 to 200° C. is 0.8 or less, and a dispersed diameter of the release agent is 0.1 times or less shorter than a volume average particle diameter of the colored particle.

**8 Claims, 1 Drawing Sheet**



FIG. 1



FIG. 2



**1**  
**TONER FOR DEVELOPING  
ELECTROSTATIC IMAGE**

TECHNICAL FIELD

The present invention relates to a toner for developing electrostatic to be used in electrophotography, electrostatic recording, electrostatic printing, magnetic recording, and the like for developing latent images having electrostatic properties, such as an electrostatic latent image and a magnetic latent image. Particularly, the present invention relates to a toner for developing electrostatic image (hereinafter, also simply referred to as a "toner") suitable for use in a heat-pressure fixing system such as heat roller fixing or the like.

BACKGROUND ART

Electrophotography is a technique for obtaining images by developing an electrostatic latent image formed on a photosensitive member with a toner for developing electrostatic latent image comprising a colored particle and, if necessary, one or more kinds of other particles such as an external additive and/or a carrier, transferring the toner onto a recording medium such as paper or an OHP sheet, and fixing the transferred toner onto the recording medium so as to obtain a printed product.

In the case of full-color electrophotography, colors are generally reproduced using three color toners of primary colors, yellow, magenta, and cyan or four color toners of these three colors and black to form color images. For example, in the case of color copy, an original color document is scanned, broken into a plurality of pixels, and converted into digital image signals for different colors, and then a charged photosensitive member is irradiated with light corresponding to the digital image signal for each color to form an electrostatic latent image. Then, the electrostatic latent image for a first color is developed with a toner of the first color on the photosensitive member, and a resulting toner image is transferred onto a recording medium such as paper or an OHP film. These developing and transfer steps are repeated for a second color, a third color, and, if necessary, a fourth color to superimpose color images on top of each other on the same recording medium while these color images are adjusted to their respective correct positions. In the case of color printing, digital signals for four colors are directly transmitted from, for example, a computer to a photosensitive member to separately form electrostatic latent images for four different colors. Then, development is carried out for each color and a resulting toner image is transferred onto a recording medium in the same manner as in the case of color copy. After the completion of development with all the four color toners and transfer, the toner images of four colors are fixed onto the recording medium by one-time fixing to form a full-color image.

Known methods for fixing toner images include heating, pressing, heating and pressing, and exposure to solvent vapor. Among them, a heating and pressing method using a heat roller is most widely used.

Here, in the field of such electrophotography, particularly in color electrophotography using two or more color toners, there is a strong demand for higher printing speed and lower energy for fixing. Therefore, a toner is required to have a low minimum fixing temperature and a high hot offset generation temperature. In addition, sharpness of an image formed at a higher printing speed with lower fixing energy is of growing importance.

**2**

It is generally known that a reduction in the glass transition temperature or melt viscosity of a toner is effective at lowering its minimum fixing temperature.

However, such a method may cause the following various problems: (1) the shelf stability of a toner is impaired; (2) a toner remaining on a photosensitive member forms a thin film, that is, filming occurs; (3) the maximum number of sheets that can be printed is reduced due to the occurrence of fog or filming and the printing durability of a toner is reduced; and (4) a hot offset phenomenon (hereinafter, simply referred to as "hot offset") occurs at low temperature so that part of a toner forming a toner image transferred onto a recording medium is attached to a heat roller and is then again transferred onto a subsequent recording medium.

Such hot offset is conventionally prevented by applying silicone oil onto a fixing roller.

However, such a method makes it difficult to reduce the size and price of a fixing unit (e.g. an image-forming apparatus). In addition, there is also a problem that an obtained image is too glossy.

In recent years, from the viewpoint of improving the low-temperature fixability of a toner and preventing the occurrence of hot offset, toner has been studied by focusing attention on its viscoelasticity.

For example, Japanese Patent Application Laid-Open (JP-A) No. 2004-151638 discloses a color toner for developing electrostatic image, which is designed to have excellent low-temperature fixability, high resistance to hot offset and excellent shelf stability. This color toner for developing electrostatic image comprises at least a binder resin, a colorant, and a charge control agent, and has the following dynamic viscoelastic characteristics as measured at a frequency of 10 Hz and a strain of 1%: a storage modulus at 80°C. (G'80) from  $5 \times 10^6$  to  $5 \times 10^8$  Pa; a storage modulus at 160°C. (G'160) from  $1 \times 10^2$  to  $1 \times 10^4$  Pa; a maximum value of loss tangent ( $\tan \delta$ ) from 1.2 to 2.5 in the range from 80 to 100°C.; and a minimum value of  $\tan \delta$  of 1 to 2 in the range from 95 to 125°C., and further has a volume average particle diameter (D<sub>v</sub>) from 2 to 11  $\mu\text{m}$ , and a ratio between volume average particle diameter (D<sub>v</sub>) and number average particle diameter (D<sub>p</sub>) (i.e. D<sub>v</sub>/D<sub>p</sub>) of 1.3 or less.

Further, JP-A No. Hei. 5-100477 discloses a toner designed to have excellent low-temperature fixability and offers resistance to offset over a wide temperature range. The toner comprises at least a binder resin having, as dynamic viscoelastic behaviors, a dynamic loss G'' at 150°C. of  $1 \times 10^5$  dyn/cm<sup>2</sup> or less and a dynamic modulus G' at 200°C. of  $2 \times 10^4$  dyn/cm<sup>2</sup> or more and a release agent having a melt viscosity at 140°C. from 5 to 100 cps, and has a loss tangent ( $\tan \delta$ ) in the range from 150 to 200°C. from 0.05 to 1.0.

DISCLOSURE OF THE INVENTION

These toners disclosed in JP-A No. 2004-151638 and JP-A No. Hei. 5-100477 have improved low-temperature fixability and resistance to hot offset (i.e. a higher hot offset generation temperature). However, there is still a demand for further improvement in low-temperature fixability and resistance to hot offset. In addition, there is also a demand for improvement in not only low-temperature fixability and resistance to hot offset but also other various properties.

It is therefore an object of the present invention to provide a toner for developing electrostatic image which shows excellent fixability over a wide temperature range including a low temperature range, has high resistance to hot offset, and is further excellent in shelf stability, cleaning properties on a photosensitive member, and printing durability.

In order to achieve the above object, the present inventors have made an extensive study, and as a result found that the above object can be achieved by a toner which comprises a toner particle containing a release agent finely dispersed therein, and which has a specific loss tangent-temperature relationship.

Based on the above findings, the present invention is directed to a toner for developing electrostatic image comprising a colored particle containing a binder resin, a colorant and a release agent, wherein the toner for developing electrostatic image has two or more maximum values of peaks or shoulders of loss tangent ( $\tan \delta$ ) in the range from 50 to 120° C., a loss tangent ( $\tan \delta$ ) in the range from 100 to 200° C. is 0.8 or less, and a dispersed diameter of the release agent is 0.1 times or less shorter than a volume average particle diameter of the colored particle.

It is preferable that the toner for developing electrostatic image has a ratio of a loss tangent at 150° C. ( $\tan \delta$  (150° C.)) and a loss tangent at 200° C. ( $\tan \delta$  (200° C.)) (i.e.,  $\tan \delta$  (200° C.)/ $\tan \delta$  (150° C.)) of 1.2 or more.

It is also preferable that the shape factors SF-1 and SF-2 of the colored particle in the toner for developing electrostatic image are  $130 \leq SF-1 \leq 170$  and  $110 \leq SF-2 \leq 150$ .

It is also preferable that the toner for developing electrostatic image is produced by a polymerization method.

It is also preferable that a volume average particle diameter ( $D_v$ ) of the colored particle is in the range from 4 to 10  $\mu\text{m}$ .

It is also preferable that the release agent is a multifunctional ester compound.

Another aspect of the present invention is directed to an image-forming method comprising steps of: a developing process to form a visible image with the above-described toner for developing electrostatic image on a photosensitive member; a transferring process to form a transferred image by transferring the visible image on a recording medium; and a fixing process to fix the transferred image.

The toner according to the present invention shows excellent fixability over a wide temperature range including a low temperature range, has high resistance to hot offset, and is further excellent in shelf stability, cleaning properties on a photosensitive member, and printing durability.

#### BRIEF DESCRIPTION OF THE DRAWINGS

In the accompanying drawings,

FIG. 1 is a graph which shows one example of the relationship between the loss tangent ( $\tan \delta$ ) of a toner according to the present invention and temperature; and

FIG. 2 is an illustration which shows one example of the structure of an image-forming apparatus using the toner for developing electrostatic image according to the present invention.

The sign in each figure refers to the following: 1: photosensitive drum, 5: charging roller, 9: transfer roller, 7: light irradiation device, 11: recording medium, 13: developing roller, 15: blade for the developing roller, 17: supply roller, 18: stirring vane, 19: toner, 21: developing device, 23: casing, 23a: toner vessel, 25: cleaning blade, 27: fixing device, 27a: heat roller, and 27b: support roller.

#### BEST MODE FOR CARRYING OUT THE INVENTION

Hereinbelow, a toner for developing electrostatic image according to the present invention will be described.

The toner for developing electrostatic image according to the present invention comprises a colored particle containing

a binder resin, a colorant and a release agent, and has two or more maximum values of peaks or shoulders of loss tangent ( $\tan \delta$ ) in the range from 50 to 120° C. and a loss tangent ( $\tan \delta$ ) in the range from 100 to 200° C. of 0.8 or less, wherein a dispersed diameter of the release agent is 0.1 times or less shorter than a volume average particle diameter of the colored particle.

In the present invention, the term "peak" refers to a region from the leading to trailing edge of a mountain-shaped curve having a maximum value, and the term "shoulder" refers to an incomplete peak which is not completely separated from the peak, that is, a stepped portion appearing in the peak region and having a maximum value.

The toner for developing electrostatic image of the present invention comprises a colored particle, and if necessary, the toner may further comprise one or more kinds of other particles or components such as an external additive to be attached to the surface of the colored particle and/or a carrier particle for carrying the colored particle.

The colored particle in the toner contains at least a binder resin, a colorant and a release agent, and if necessary, the colored particle may further contain one or more other components such as a charge control agent or the like.

As the binder resin contained in the colored particle include resins conventionally used as a binder resin for toner. For example, there may be styrene such as polystyrene, polyvinyl toluene or the like, and a polymer of derivative substitution thereof; a styrene copolymer such as a styrene-methyl acrylate copolymer, a styrene-ethyl acrylate copolymer, a styrene-butyl acrylate copolymer, a styrene-2-ethylhexyl acrylate copolymer, a styrene-methyl methacrylate copolymer, a styrene-ethyl methacrylate copolymer, a styrene-butyl methacrylate copolymer, a styrene-butadiene copolymer or the like; polymethyl methacrylate, polyester, an epoxy resin, polyvinyl butyral, an aliphatic or alicyclic hydrocarbon resin, polyolefin, a (meth)acrylate resin, a norbornene-based resin and a hydrogenated product of the styrene-based resin.

Examples of the colorant include various pigments and dyes such as carbon black, titanium black, magnetic powders (magnetic materials), oil black, titanium white or the like.

In the case of producing a black toner, carbon black may be preferably used. A primary particle diameter of carbon black which is suitably used is 20 to 40 nm. By using colorant having such a primary particle diameter, it is possible to uniformly disperse the carbon black in the toner, thereby suppressing the occurrence of fog.

In the case of producing a full-color toner, a yellow colorant, a magenta colorant and a cyan colorant are usually used.

As the yellow colorant, a compound such as an azo-based pigment, a condensed polycyclic pigment or the like may be used. Specific examples of such a yellow colorant include C.I. Pigment Yellow 3, 12, 13, 14, 15, 17, 62, 65, 73, 74, 75, 83, 90, 93, 97, 120, 138, 155, 180, 181, 185, 186 and so on.

As the magenta colorant, a compound such as an azo-based pigment, a condensed polycyclic pigment or the like may be used. Specific examples of such a magenta colorant include C.I. Pigment Red 31, 48, 57, 58, 60, 63, 64, 68, 81, 83, 87, 88, 89, 90, 112, 114, 122, 123, 144, 146, 149, 150, 163, 170, 184, 185, 187, 202, 206, 207, 209, and 251, C.I. Pigment Violet 19 and so on.

As the cyan colorant, a phthalocyanine compound such as a copper phthalocyanine compound or a derivative thereof, an anthraquinone compound or the like may be used. Specific examples of such a cyan colorant include C.I. Pigment Blue 2, 3, 6, 15, 15:1, 15:2, 15:3, 15:4, 16, 17, 60 and so on.

The amount of each of the colorants to be used is preferably 1 to 10 parts by weight with respect to 100 parts by weight of the binder resin.

Examples of the magnetic materials include iron oxides such as magnetite,  $\gamma$ -iron oxide, ferrite, iron-excess ferrite or the like; iron, cobalt or nickel, or alloys thereof with one or more of aluminum, cobalt, copper, lead, magnesium, tin, zinc, antimony, beryllium, bismuth, cadmium, calcium, manganese, selenium, titanium, tungsten and vanadium, or mixtures thereof.

The magnetic material is usually used in an amount from 10 to 60 parts by weight, preferably 20 to 50 parts by weight, with respect to 100 parts by weight of the binder resin.

Examples of the release agent include: polyolefin waxes such as low-molecular weight polyethylene, low-molecular weight polypropylene, low-molecular weight polybutylene or the like; natural waxes such as candelilla wax, carnauba wax, rice wax, Japan wax, jojoba wax or the like; petroleum waxes such as paraffin, microcrystalline, petrolatum or the like and modified waxes thereof; synthetic waxes such as Fischer-Tropsch wax or the like; and multifunctional ester compounds such as pentaerythritol tetra-myristate, pentaerythritol tetrastearate, pentaerythritol tetrapalmitate, dipentaerythritol hexamyrystate, dipentaerythritol hexastearate or the like.

These release agents can be used alone or in combination of two or more kinds.

Among these release agents, synthetic waxes and multifunctional ester compounds are preferably used. Among them, from the viewpoint of obtaining a toner offering an excellent balance between fixability and releasability upon fixing, multifunctional ester compounds whose endothermic peak temperature during temperature rise in a DSC curve measured using a differential scanning calorimeter is preferably in the range from 30 to 150°C., more preferably in the range from 40 to 100°C., most preferably in the range from 50 to 80°C., are preferably used. Particularly, multifunctional ester compounds having a molecular weight of 1,000 or more, being soluble in styrene in an amount of 5 parts by weight or more with respect to 100 parts by weight of styrene at 25°C., and having an acid value of 10 mgKOH/g or less are more preferably used because such a multifunctional ester compounds have a significant effect on lowering the minimum fixing temperature. Herein, the term "endothermic peak temperature" means a value measured in accordance with ASTM D3418-82.

In the present invention, the dispersed diameter of the release agent is 0.1 times or less shorter than the volume average particle diameter of the colored particle. The release agent may be so finely dispersed in the colored particle that the existence thereof cannot or can hardly be recognized with a transmission electron microscope (TEM). It is to be noted that a state where the release agent is finely dispersed in the colored particle includes a state where the release agent and the binder resin contained in the colored particle are mutually dissolved.

If the dispersed diameter of the release agent exceeds 0.1 times the volume average particle diameter of the colored particle, there is a fear that bleeding may occur during high-temperature storage, thereby impairing shelf stability and causing poor printing.

The term "dispersed diameter of the release agent" herein refers to a dispersed diameter of the release agent as measured in the following manner. The toner is dispersed in an epoxy resin, cured, cooled to a temperature of -80°C., and cut with a microtome to prepare a thin slice. The thin slice is stained with a vapor of 0.5% aqueous solution of ruthenium tetroxide

for about 5 minutes, and then the stained thin slice is observed with a TEM (transmission electron microscope) (magnification:  $\times 5,000$  to  $\times 6,000$ ).

The concentration of the toner in a sample obtained by dispersing the toner in an epoxy resin is adjusted so that 5 to 10 cross-sections of the colored particles can be observed in a TEM image covering an area of 28 $\times$ 35  $\mu\text{m}$ . Among the colored particles observed in the TEM image covering an area of 28 $\times$ 35  $\mu\text{m}$ , one whose cross-section is not entirely shown and one whose cross-sectional size is not 0.6 to 1.2 times the volume average particle diameter of the colored particle are excluded from evaluation. The cross-sections of the colored particles other than such colored particles excluded from evaluation are observed on the TEM screen to determine the diameters of island-shaped separate phases of the release agent. The average diameter of the island-shaped separate phases is defined as a dispersed diameter of the release agent.

The release agent is usually used in an amount from 0.5 to 50 parts by weight, preferably 1 to 20 parts by weight, with respect to 100 parts by weight of the binder resin.

The colored particle preferably contains a charge control agent. The charge control agent is not particularly limited, and examples thereof include charge control agents conventionally used for toner. Among these charge control agents, charge control resins are preferably used because they are highly compatible with binder resins and colorless, and make it possible to provide a toner whose charge property is stable even at high-speed color continuous printing.

Such charge control resins include a negative charge control resin and a positive charge control resin, and which one is used depends on whether the toner according to the present invention is prepared as a positively chargeable toner or a negatively chargeable toner. Hereinbelow, the negative charge control resin and the positive charge control resin will be described.

Examples of the negative charge control resin include resins having, in the side chain of a polymer, a substituent selected from the group consisting of a carboxyl group or a salt thereof, a phenol group or a salt thereof, a thiophenol group or a salt thereof, a sulfonic acid group or a salt thereof.

Among these negative charge control resins, resins having, in the side chain of a polymer, a sulfonic acid group or a salt thereof are preferably used. Specific examples of such a negative charge control resin include resins obtained by copolymerizing a monovinyl monomer containing a sulfonic acid group or a salt thereof and another monovinyl monomer copolymerizable with the monovinyl monomer containing a sulfonic acid group or a salt thereof. Examples of another monovinyl monomer copolymerizable with a monovinyl monomer containing a sulfonic acid group or a salt thereof include ethylenically unsaturated carboxylic acid ester monomers, aromatic vinyl monomers, ethylenically unsaturated nitrile monomers and so on.

Examples of the monovinyl monomer containing a sulfonic acid group or a salt thereof include styrene sulfonic acid, sodium styrene sulfonate, potassium styrene sulfonate, 2-acrylamido-2-methylpropanesulfonic acid, sodium vinyl sulfonate, ammonium methacryl sulfonate or the like.

Examples of the ethylenically unsaturated carboxylic acid ester monomer include methyl(meth)acrylate, ethyl (meth)acrylate, propyl(meth)acrylate, butyl (meth)acrylate, 2-ethyl-hexyl(meth)acrylate or the like. The term "(meth)acrylate" refers to either acrylate or methacrylate.

Examples of the aromatic vinyl monomer include styrene, methyl styrene, vinyl toluene, chlorostyrene, hydroxymethyl styrene or the like.

Examples of the ethylenically unsaturated nitrile monomer include (meth)acrylonitrile, fumaronitrile,  $\alpha$ -chloroacrylonitrile,  $\alpha$ -cyanoethylacrylonitrile or the like.

An amount of the monovinyl monomer containing a functional group such as a sulfonic acid group or a salt thereof in the negative charge control resin is preferably in the range from 0.5 to 15 wt %, more preferably in the range from 1 to 10 wt %. If the amount of such a monovinyl monomer contained in the negative charge control resin is less than the above lower limit value, the charge property of the toner and the dispersibility of the colorant may be poor, thereby lowering printing density and transparency. If the amount of such a monovinyl monomer contained in the negative charge control resin exceeds the above upper limit value, a reduction in the charge amount of the toner under high-temperature and high-humidity conditions may be increased, thereby causing fog.

The weight average molecular weight of the negative charge control resin is preferably in the range from 2,000 to 50,000, more preferably in the range from 4,000 to 40,000, most preferably in the range from 6,000 to 35,000.

The glass transition temperature of the negative charge control resin is preferably in the range from 40 to 80°C., more preferably in the range from 45 to 75°C., most preferably in the range from 45 to 70°C. If the glass transition temperature of the negative charge control resin is less than the above lower limit value, the shelf stability of the toner may be impaired. If the glass transition temperature of the negative charge control resin exceeds the above upper limit value, the fixability of the toner may be deteriorated.

Examples of the positive charge control resin include: resins containing an amino group such as  $-\text{NH}_2$ ,  $-\text{NHCH}_3$ ,  $-\text{N}(\text{CH}_3)_2$ ,  $-\text{NHC}_2\text{H}_5$ ,  $-\text{N}(\text{C}_2\text{H}_5)_2$ ,  $-\text{NHC}_2\text{H}_4\text{OH}$  or the like; and resins containing, as a functional group, an ammonium salt of the above-mentioned amino group. These resins can be obtained by, for example, copolymerizing a monovinyl monomer containing an amino group with a monovinyl monomer copolymerizable with the monovinyl monomer containing an amino group. Thus obtained copolymer may be modified to obtain an ammonium salt thereof. Alternatively, these resins may also be obtained by copolymerizing a monovinyl monomer containing an ammonium salt group with a monovinyl monomer copolymerizable with the monovinyl monomer containing an ammonium salt group. However, a method for obtaining a positive charge control resin is not limited to these methods. Examples of the monovinyl monomer copolymerizable with a monovinyl monomer containing an amino group and the monovinyl monomer copolymerizable with a monovinyl monomer containing an ammonium salt group include those used for obtaining a negative charge control resin.

Examples of the monovinyl monomer containing an amino group include: alkyl(meth)acrylamide monomers such as (meth)acrylamide, N-methyl(meth)acrylamide, N,N-dimethyl(meth)acrylamide, N-ethyl(meth)acrylamide or the like; (meth)acrylic acid derivatives such as 3-(dimethylamino)propyl(meth)acrylate; allylamine or the like; and styrene derivatives such as 2-aminostyrene, 4-aminostyrene or the like.

An amount of the monovinyl monomer, having a functional group such as an amino group, an ammonium salt group or the like, contained in the positive charge control resin is preferably in the range from 0.5 to 15 wt %, more preferably in the range from 1 to 10 wt %. If the amount of the monovinyl monomer, having a functional group such as an amino group or an ammonium salt group, contained in the positive charge control resin is less than the above lower limit value, the charge property of the toner and the dispersibility of the colorant may be poor, thereby lowering printing density

and transparency. If the amount of the monovinyl monomer, having a functional group such as an amino group or an ammonium salt group, contained in the positive charge control resin exceeds the above upper limit value, a reduction in the charge amount of the toner under high-temperature and high-humidity conditions may be increased, thereby causing fog.

The weight average molecular weight of the positive charge control resin is preferably in the range from 2,000 to 30,000, more preferably in the range from 4,000 to 25,000, most preferably in the range from 6,000 to 20,000.

The glass transition temperature of the positive charge control resin is preferably in the range from 40 to 100°C., more preferably in the range from 45 to 80°C., most preferably in the range from 45 to 70°C. If the glass transition temperature of the positive charge control resin is less than the above lower limit value, the shelf stability of the toner may be impaired. If the glass transition temperature of the positive charge control resin exceeds the above upper limit value, the fixability of the toner may be deteriorated.

In the toner of the present invention, the negative charge control resin and the positive charge control resin may be used together, and the ratio between the amounts of these resins to be used varies depending on whether the toner is prepared as a negatively chargeable toner or a positively chargeable toner. In the case of producing a negatively chargeable toner, the ratio between the amounts of the negative and positive charge control resins to be used is controlled so that the molar equivalent of a functional group (e.g. a sulfonic acid group) contained in the negative charge control resin to provide negatively charging ability is larger than that of a functional group (e.g. a quaternary ammonium salt group) contained in the positive charge control resin to provide positively charging ability. Conversely, in the case of producing a positively chargeable toner, the ratio between the amounts of the negative and positive charge control resins to be used is controlled so that the molar equivalent of a functional group contained in the positive charge control resin is larger than that of a functional group contained in the negative charge control resin.

An amount of the charge control resin to be used is preferably in the range from 0.01 to 30 parts by weight, more preferably in the range from 0.3 to 25 parts by weight, with respect to 100 parts by weight of the polymerizable monomer to be used for obtaining a binder resin.

The colored particle may be a so-called core-shell structured particle obtained by using two different polymers for forming an inner part (i.e. a core layer) of the particle and an outer part (i.e. a shell layer) of the toner, respectively. A core-shell structured particle obtained by covering an inner part (i.e. a core layer) made of a substance having a low softening point with a substance having a softening point higher than that of the inner part is preferably used because such a core-shell structured particle can strike a balance between the low-temperature fixability and the shelf stability of the toner.

The core layer of the core-shell structured particle usually comprises the binder resin, colorant and release agent, and if necessary the charge control resin and/or one or more other additives. On the other hand, the shell layer is usually composed of only a binder resin.

In the case of the core-shell structured particle, the glass transition temperature of a polymer constituting the core layer is preferably in the range from 0 to 80°C., more preferably in the range from 40 to 60°C. If the glass transition temperature of the polymer exceeds 80°C., the minimum fixing temperature of the toner may be increased. On the other

hand, if the glass transition temperature of the polymer is less than 0° C., the shelf stability of the toner may be impaired.

It is necessary to set the glass transition temperature of a polymer constituting the shell layer to be higher than that of the polymer constituting the core layer. From the view point of improving the shelf stability of the toner, the glass transition temperature of a polymer constituting the shell layer is preferably in the range from 50 to 130° C., more preferably in the range from 60 to 120° C., most preferably in the range from 80 to 110° C. If the glass transition temperature of the polymer is less than the above lower limit value, the shelf stability of the toner may be impaired. On the other hand, if the glass transition temperature of the polymer exceeds the above upper limit value, the fixability of the toner may be deteriorated.

The difference in the glass transition temperature between the polymer constituting the core layer and the polymer constituting the shell layer is preferably 10° C. or more, more preferably 20° C. or more, most preferably 30° C. or more. If the difference in the glass transition temperature between these polymers is less than the above lower limit value, a balance between the shelf stability and the fixability of the toner may be decreased.

The weight ratio between the core layer and the shell layer of the core-shell structured particle is not particularly limited, but is preferably in the range from 80/20 to 99.9/0.1 (core layer/shell layer). If the weight ratio of the shell layer is less than the above lower limit value, the shelf stability of the toner may be impaired. To the contrary, if the weight ratio of the shell layer exceeds the above upper limit value, low-temperature fixing may be difficult to be carried out.

The average thickness of the shell layer of the core-shell structured particle is usually in the range from 0.001 to 1.0  $\mu\text{m}$ , preferably in the range from 0.003 to 0.5  $\mu\text{m}$ , more preferably in the range from 0.005 to 0.2  $\mu\text{m}$ . If the average thickness of the shell layer exceeds the above upper limit value, the fixability of the toner may be deteriorated. If the average thickness of the shell layer is less than the above lower limit value, the shelf stability of the toner may be impaired.

When the core layer and the shell layer of the core-shell structured particle can be observed with an electron microscope, the particle diameter of the core layer and the thickness of the shell layer can be determined by randomly selecting a core-shell structured particle in an electron micrograph and directly measuring the size of the core layer particle and the thickness of the shell layer of the core-shell structured particle. On the other hand, when it is difficult to observe the core layer particle and the shell layer with an electron microscope, the thickness of the shell layer can be determined by calculating from the particle diameter of the core layer and the amount of a polymerizable monomer for shell used for forming the toner.

The volume average particle diameter (Dv) of the colored particle is preferably in the range from 4 to 10  $\mu\text{m}$ , more preferably in the range from 5 to 8  $\mu\text{m}$ . If the Dv is less than 4  $\mu\text{m}$ , the toner may leak from a sealing portion to make the inside of an image-forming apparatus dirty, the flowability of the toner may be deteriorated so that fog may occur, the toner may remain with inferior transferability, or the cleaning property of the toner may be lowered. On the other hand, if the Dv exceeds 10  $\mu\text{m}$ , thin line reproducibility may be lowered and therefore high image quality may not be able to be achieved, or fixability of the toner may be deteriorated.

The colored particle usually has a ratio between its volume average particle diameter (Dv) and number average particle diameter (Dp) (i.e. Dv/Dp) from 1 to 1.3, preferably 1 to 1.2.

If the Dv/Dp exceeds the above upper limit value, transferability may be deteriorated, fog may occur, or the production yield of the toner may be lowered.

The shape factors SF-1 and SF-2 of the colored particle are preferably  $130 \leq \text{SF-1} \leq 170$  and  $110 \leq \text{SF-2} \leq 150$ , respectively, from the viewpoint of achieving excellent transferability and cleaning property.

In the present invention, the shape factors SF-1 and SF-2 are defined by the following formulas:

$$(\text{SF-1}) = (L_{\text{MAX}}^2/S) \times (\pi/4) \times 100$$

$$(\text{SF-2}) = (R^2/S) \times (4/\pi) \times 100$$

wherein,  $L_{\text{MAX}}$  is an absolute maximum length of a projected image, S is a projected area of the projected image, and R is a length of perimeter of the projected image.

Of these shape factors SF-1 and SF-2, SF-1 represents the degree of distortion of the whole particle, and SF-2 represents the degree of unevenness of a small part of the particle. It is to be noted that in the present invention, when an external additive is attached to the surface of the colored particle, the shape factor of the colored particle can be determined based on a projected image of the colored particle to which an external additive is attached. In the case of a two-component toner, a shape factor is determined based on a projected image of a colored particle contained in the toner.

The toner of the present invention may contain an external additive. By adhering or embedding an external additive to or in the surface of the colored particle, it is possible to control the charge property, flowability, and shelf stability of the colored particle.

Such an external additive is not particularly limited, and examples thereof include external additives conventionally used for a toner, such as inorganic particles and organic resin particles. Specific examples of the inorganic particles include silica, aluminum oxide, titanium oxide, zinc oxide and tin oxide. Specific examples of the organic resin particles include (meth)acrylic acid ester polymer particles, styrene-(meth)acrylic acid ester copolymer particles or the like. Among these external additives, silica or titanium oxide is suitably used. These particles whose surface has been subject to hydrophobicity-imparting treatment are preferably used, and silica particles subject to hydrophobicity-imparting treatment are particularly preferably used.

An amount of the external additive is not particularly limited, but is usually in the range from 0.1 to 6 parts by weight with respect to 100 parts by weight of the colored particle. The external additive can be used in combination of two or more kinds. In the case of using two or more kinds together, a combination of inorganic particles having different average particle diameters or a combination of an inorganic particle and an organic resin particle is suitable. Adhesion of the external additive to the toner particles is usually achieved by mixing the external additive and the colored particles in a mixer such as HENSCHEL MIXER (trade name) or the like.

In a case where the toner of the present invention is prepared as a two-component toner, the toner contains a carrier. The carrier for carrying the colored particle is not particularly limited, and examples thereof include carriers conventionally used for toner, such as magnetic powders (e.g. iron powder, ferrite powder or nickel powder), glass beads, and these carriers whose surfaces have been treated with a fluorine-based resin, a styrene/acrylic resin or a silicon-based resin and so on.

In the case of the two-component toner, the concentration of the colored particle in the toner is usually in the range from

## 11

0.1 to 50 wt %, preferably in the range from 0.5 to 15 wt %, more preferably in the range from 3 to 5 wt %.

The toner of the present invention has two or more maximum values of peaks or shoulders of loss tangent ( $\tan \delta$ ) in the range from 50 to 120° C., preferably in the range from 55 to 100° C., more preferably in the range from 60 to 95° C., and has a loss tangent ( $\tan \delta$ ) in the range from 100 to 200° C. of 0.8 or less. FIG. 1 shows an example of such a loss tangent ( $\tan \delta$ ).

The toner having two or more maximum values of peaks or shoulders of loss tangent ( $\tan \delta$ ) in the range from 50 to 120° C. and a loss tangent ( $\tan \delta$ ) in the range from 100 to 200° C. of 0.8 or less has excellent low-temperature fixability and a high hot offset generation temperature. Therefore, even when such a toner is used for printing a large number of sheets, filming is less likely to occur, and the toner exhibits excellent printing durability.

The toner preferably has a ratio between a loss tangent at 150° C. ( $\tan \delta$  (150° C.)) and a loss tangent at 200° C. ( $\tan \delta$  (200° C.)) (i.e.  $\tan \delta$  (200° C.)/ $\tan \delta$  (150° C.)) of 1.2 or more because the above-described effects of the toner are further enhanced.

It is to be noted that the loss tangent ( $\tan \delta$ ) of the toner is the ratio between a loss modulus ( $G''$ ) and a storage modulus ( $G'$ ) (i.e.  $G''/G'$ ) representing the viscoelastic properties of the toner.

The viscoelastic properties such as loss modulus ( $G''$ ) and storage modulus ( $G'$ ) can be measured using an instrument such as a viscoelasticity measuring instrument (rheometer) (product name: RDA-II; manufactured by Rheometrics).

The toner of the present invention described above shows excellent fixability over a wide temperature range including a low temperature range, and has high resistance to hot offset, and is further excellent in shelf stability, cleaning properties on a photosensitive member, printing durability and so on.

The colored particles can be produced by a conventional method such as a dry method (e.g. a pulverizing method or the like) or a wet method (e.g. a suspension polymerization method, an emulsion polymerization aggregation method, a dissolution suspension method, a phase inversion emulsion method or the like). Among these methods, a wet method is preferably used, and polymerization methods such as a suspension polymerization method, an emulsion polymerization aggregation method and so on are more preferably used.

Particularly, in the case of producing core-shell structured colored particle, a colored particle obtained by any one of the above methods may be used as a core layer, and the colored particle is covered with a shell layer by a conventional method such as a spray drying method, an interfacial reaction method, an in situ polymerization method, a phase separation method or the like.

Among these production methods, a polymerization method is preferably used for producing colored particle since a colored particle having an average circle degree of 1, that is, a colored particle having a shape close to a perfect sphere can be obtained. A core-shell structured colored particle is preferably produced by covering a colored particle produced by a polymerization method with a shell layer by an in situ polymerization method.

Hereinbelow, a method for producing core-shell structured colored particle, in which a colored particle as a core layer is produced by a polymerization method and the colored particle is covered with a shell layer by an in situ polymerization method, will be described.

First, a colored particle as a core layer is produced in the following manner. A colorant, a release agent, and if necessary, a charge control agent and/or other additives are dis-

## 12

solved or dispersed in a polymerizable monomer as a raw material of a binder resin to prepare a polymerizable monomer composition. Then, the polymerizable monomer composition is added to an aqueous dispersion medium containing a dispersion stabilizer to form droplets of the polymerizable monomer composition. A polymerization initiator is added to the dispersion liquid containing the droplets to carry out polymerization, and if necessary, resulting particles are aggregated with each other, followed by filtration, washing, dewatering, and drying to obtain colored particle.

The polymerizable monomer as a raw material of a binder resin contains, as a main component, a monovinyl monomer, and if necessary, as a sub-component, a cross-linkable monomer, a cross-linkable polymer, and other monomers. Such a polymerizable monomer is polymerized to be a binder resin component contained in the colored particle.

Examples of the monovinyl monomer include: aromatic vinyl monomers such as styrene, vinyl toluene,  $\alpha$ -methyl styrene or the like; (meth)acrylic monomers such as (meth) acrylic acid, methyl(meth)acrylate, ethyl (meth)acrylate, propyl(meth)acrylate, butyl (meth)acrylate, 2-ethylhexyl(meth) acrylate, cyclohexyl (meth)acrylate, isobonyl(meth)acrylate, dimethylaminoethyl(meth)acrylate, (meth)acrylamide or the like; and monoolefin-based monomers such as ethylene, propylene, butylene or the like. It is to be noted that in the present invention, the term "(meth)acrylic" refers to either acrylic or methacrylic, and the term "(meth)acrylate" refers to either acrylate or methacrylate.

These monovinyl monomers can be used alone or in combination of two or more kinds. Among these monovinyl monomers, an aromatic vinyl monomer alone or a combination of an aromatic vinyl monomer and a (meth)acrylic monomer is suitably used.

By using the monovinyl monomer together with a cross-linkable monomer and a cross-linkable polymer, it is possible to effectively improve hot offset.

The cross-linkable monomer herein refers to a monomer having two or more polymerizable carbon-carbon unsaturated double bonds. Examples of such a monomer include: aromatic divinyl compounds such as divinylbenzene, divinyl-naphthalene, and derivatives thereof; compounds having two vinyl groups in a molecule including di(meth)acrylic acid esters such as ethylene glycol dimethacrylate, diethylene glycol dimethacrylate or the like, divinyl ethers or the like; compounds having three or more vinyl groups in a molecule such as pentaerythritol triallyl ether, trimethylolpropane triacrylate or the like.

The cross-linkable polymer herein refers to a polymer having two or more vinyl groups. Specific examples of such a polymer include esters obtained by condensation between a polymer having two or more hydroxyl groups in a molecule (e.g. polyethylene, polypropylene, polyester, polyethylene glycol or the like) and an unsaturated carboxylic acid monomer (e.g. acrylic acid, methacrylic acid or the like).

The cross-linkable monomer and cross-linkable polymer can be used alone or in combination of two or more kinds. An amount thereof to be used is usually 10 parts by weight or less, preferably 0.1 to 2 parts by weight, with respect to 100 parts by weight of the monovinyl monomer.

As other monomers, a radically polymerizable epoxy compound or a radically polymerizable acid halide can be used to improve the dispersibility of the colorant, to prevent reaggregation of the colorant, and to control the dispersion of the release agent.

Examples of the radically polymerizable epoxy compound include glycidyl methacrylate, glycidyl acrylate, allyl glycidyl ether, styryl glycidyl ether, epoxy resins or the like.

Examples of the radically polymerizable acid halide include chloride compounds such as acryl chloride, methacryl chloride, styrene carbonyl chloride, styrene sulfonyl chloride, 2-methacryloyloxy ethyl succinyl chloride, 2-methacryloyloxy ethyl hexahydrophthalyl chloride or the like; and bromide compounds such as acryl bromide, methacryl bromide, styrene carbonyl bromide, styrene sulfonyl bromide, 2-methacryloyloxy ethyl succinyl bromide, 2-methacryloyloxy ethyl hexahydrophthalyl bromide or the like.

In the case of using such a radically polymerizable epoxy compound or acid halide, an amount thereof to be added to the polymerizable monomer used for forming a binder resin component is preferably in the range from 0.1 to 5 wt %, more preferably in the range from 0.2 to 3 wt %. If the amount of the radically polymerizable epoxy compound or acid halide is less than 0.1 wt %, the effect of dispersing a pigment may not be able to be satisfactorily obtained. If the amount of the radically polymerizable epoxy compound or acid halide contained exceeds 5 wt %, hot offset may occur. In either case, there is a possibility that image quality is lowered.

These radically polymerizable epoxy compounds and acid halides can be used alone or in combination of two or more kinds.

Examples of the dispersion stabilizer include well-known surfactants, inorganic dispersants, and organic dispersants. Among them, inorganic dispersants are preferably used as they can be easily removed by after treatment. Specific examples of the inorganic dispersant include: inorganic salts such as barium sulfate, calcium carbonate, calcium phosphate or the like; inorganic oxides such as silica, aluminum oxide, titanium oxide or the like; and inorganic hydroxides such as aluminum hydroxide, magnesium hydroxide, ferric hydroxide or the like. Among these dispersion stabilizers, those containing a colloid of a hardly water-soluble inorganic hydroxide are particularly preferably used since they can narrow the particle diameter distribution of the polymer particles, hardly remain after washing dispersion stabilizer, and contribute to reproduction of a sharp image.

The dispersion stabilizer is usually used in an amount from 0.1 to 20 parts by weight with respect to 100 parts by weight of the polymerizable monomer. By setting the amount of the dispersion stabilizer to a value within the above range, it is possible to carry out polymerization sufficiently stably while suppressing the aggregation of the polymer, and as a result a toner having a desired particle diameter can be obtained.

Examples of the polymerization initiator include: persulfates such as potassium persulfate, ammonium persulfate or the like; azo compounds such as 4,4'-azobis(4-cyanovaleic acid), 2,2'-azobis(2-methyl-N-(2-hydroxyethyl)propionamide), 2,2'-azobis(2-amidinopropane)dihydrochloride, 2,2'-azobis(2,4-dimethylvaleronitrile), dimethyl-2,2'-azobis(2-methylpropionate), 2,2'-azobisisobutyronitrile or the like; organic peroxides such as di-t-butyl peroxide, dicumyl peroxide, lauroyl peroxide, benzoyl peroxide, t-butylperoxy-2-ethylhexanoate, t-hexylperoxy-2-ethylhexanoate, t-butylperoxy-pivalate, di-isopropylperoxy dicarbonate, di-t-butylperoxy isophthalate, 1,1,3,3-tetramethylbutylperoxy-2-ethylhexanoate, t-butylperoxy isobutyrate or the like; and redox initiators prepared by combining these polymerization initiators with reducing agents.

Among these polymerization initiators, an oil-soluble polymerization initiator which can be dissolved in the polymerizable monomer used is preferably used. If necessary, such a polymerization initiator may be used together with a water-soluble polymerization initiator.

The polymerization initiator is used in an amount from 0.1 to 20 parts by weight, preferably 0.3 to 15 parts by weight,

more preferably 0.5 to 10 parts by weight, with respect to 100 parts by weight of the polymerizable monomer.

The polymerization initiator may be preliminarily added to the polymerizable monomer composition. However, in the case of suspension polymerization, the polymerization initiator may be directly added to a suspension obtained after the completion of the step of forming droplets of the polymerizable monomer composition, or in the case of emulsion polymerization, the polymerization initiator may be directly added to an emulsion obtained after the completion of the step of emulsification.

Further, at the time of polymerization, a molecular weight control agent is preferably added to a reaction system. Examples of the molecular weight control agent include: mercaptan compounds such as t-dodecylmercaptan, n-dodecylmercaptan, n-octylmercaptan, 2,2,4,6,6-pentamethylheptane-4-thiol or the like; and thiuram disulfide compounds such as tetramethylthiuram disulfide, tetraethylthiuram disulfide or the like. The molecular weight control agent is usually used in an amount from 0.01 to 10 parts by weight, preferably 0.1 to 5 parts by weight with respect to 100 parts by weight of the polymerizable monomer.

Next, the colored particle produced by the polymerization method described above can be covered with a shell layer in the following manner. In the case of covering with a shell layer by in situ polymerization, a polymerizable monomer for forming a shell layer (hereinafter, simply referred to as a "polymerizable monomer for shell") and a polymerization initiator for shell are added to an aqueous dispersion medium, in which the colored particle as a core layer is dispersed, to carry out polymerization, followed by filtration, washing, dewatering and drying to obtain a core-shell structured colored particle.

Specific examples of a method for forming a shell layer include: a method in which a polymerizable monomer for shell is added to a reaction system of the polymerization reaction performed to obtain a colored particle as a core layer to continuously perform polymerization; a method in which a colored particle obtained by polymerizing a polymerizable monomer, followed by association, filtration, washing, dewatering and drying is charged as a core layer into a reaction system different from that used for producing colored particle, and a polymerizable monomer for shell is added thereto to carry out polymerization stepwise; or the like.

Examples of the polymerizable monomer for shell include monomers such as styrene, acrylonitrile, methyl methacrylate or the like, capable of forming a polymer having a glass transition temperature higher than 80° C. The polymerizable monomer for shell may be preferably used alone or in combination of two or more kinds.

As the polymerization initiator for shell, a water-soluble polymerization initiator can be used. Examples of the water-soluble polymerization initiator include: persulfates such as potassium persulfate, ammonium persulfate or the like; azo-based initiators such as 2,2'-azobis(2-methyl-N-(2-hydroxyethyl)propionamide), 2,2'-azobis-(2-methyl-N-(1,1-bis(hydroxymethyl)2-hydroxyethyl)propionamide) or the like. The water-soluble polymerization initiator is usually used in an amount from 0.1 to 50 parts by weight, preferably 1 to 30 parts by weight, with respect to 100 parts by weight of the polymerizable monomer for shell.

The dispersion stabilizer contained in the aqueous dispersion of the colored particle obtained by polymerization is preferably removed by adding an acid or an alkali to the aqueous dispersion to dissolve the dispersion stabilizer in water. In a case where a colloid of a hardly water-soluble inorganic hydroxide is used as the dispersion stabilizer, an

acid is preferably added to the aqueous dispersion to adjust the pH of the aqueous dispersion to 6.5 or less. Examples of the acid to be added include inorganic acids such as sulfuric acid, hydrochloric acid, nitric acid or the like; and organic acids such as formic acid, acetic acid or the like. Particularly, among these acids, sulfuric acid may be suitably used from the viewpoint of increasing the efficiency of removing the dispersion stabilizer and lightening the load on production facilities.

The colored particle, preferably the core-shell structured colored particle, obtained by the above-described method can be used directly as a toner for developing electrostatic image, but may further be mixed with an external additive, a carrier and/or other microparticles in a high-speed agitator such as HENSCHEL MIXER (trade name).

The characteristics of the toner produced by the above-described method, such as a dispersed diameter of the release agent and a loss tangent ( $\tan \delta$ ) of the toner, are determined by interactions among the kinds and used amounts of the polymerizable monomer, the release agent and so on as well as polymerization temperature, polymerization time and so on.

The toner of the present invention can be widely used in electrophotography, electrostatic recording, electrostatic printing or the like for electrostatic latent image-developing systems, developing methods and image-forming apparatuses wherein electrostatic latent images are developed to form images such as photographs, pictures, text, symbols or the like. Particularly, the toner of the present invention is suitable for use in a heat-pressure fixing system, method and apparatus such as heat roller fixing or the like.

Hereinbelow, an image-forming method of the present invention will be described.

FIG. 2 shows one example of a structure of an image-forming apparatus using the toner for developing electrostatic latent image of the present invention. As shown in FIG. 2, the image-forming apparatus includes a photosensitive drum 1 as a photosensitive member, and the photosensitive drum 1 is provided so as to be rotatable in a direction indicated by the arrow A. The photosensitive drum 1 is obtained by providing a photoconductive layer on a conductive support drum. The photoconductive layer is formed from, for example, an organic photosensitive member, a selenium photosensitive member, a zinc oxide photosensitive member, an amorphous silicon photosensitive member or the like. Among these photosensitive members, the organic photosensitive member is preferable. The photoconductive layer may be bonded to the conductive support drum by the use of a resin. Examples of such a resin include polyester resins, acrylic resins, polycarbonate resins, phenol resins, epoxy resins or the like. Among them, the polycarbonate resins are preferable.

Around the photosensitive drum 1, there are provided, along the circumferential direction thereof, a charging roller 5 as a charging member, a light irradiation device 7 as an exposure device, a developing device 21, a transfer roller 9 and a cleaning blade 25.

On the downstream side of the photosensitive drum 1 in a conveying direction, there is provided a fixing device 27. The fixing device 27 includes a heat roller 27a and a support roller 27b.

A path for conveying a recording medium is provided so that a recording medium can pass between the photosensitive drum 1 and the transfer roller 9 and then between the heat roller 27a and the support roller 27b.

The process for forming image with the image-forming apparatus shown in FIG. 2 includes a charging step, an expo-

sure step, a developing step, a transfer step, a cleaning step, and a fixing step. These steps will be described in detail below.

The charging step is carried out to allow the surface of the photosensitive drum 1 to be uniformly positively or negatively charged using a charging member. As a charging method using the charging member, there are a contact charging method using, for example, the charging roller 5 shown in FIG. 2, a fur brush, a magnetic brush, a blade or the like, and a non-contact charging method using corona discharge. The charging method using the charging roller 5 can be replaced with such a contact charging method or a non-contact charging method.

The exposure step is carried out to form an electrostatic latent image on the surface of the photosensitive drum 1 uniformly charged. The electrostatic latent image is formed by irradiating the surface of the photosensitive drum 1 with light emitted from the light irradiation device 7 shown in FIG. 2 as an exposure device and corresponding to image signals. The light irradiation device 7 includes, for example, an irradiation device and an optical lens. Examples of the irradiation device include a laser beam irradiation device and an LED irradiation device.

The developing step is carried out by the developing device 21 to attach the toner to the electrostatic latent image formed on the surface of the photosensitive drum 1 in the exposure step. The charge polarity of the toner is selected so that the toner can be attached only to a light-radiated part in reversal development, or only to a light-non-radiated part in normal development.

The developing device 21 of the image-forming apparatus shown in FIG. 2 is designed for use in mono-component contact development. In a casing 23 for receiving the toner 19, there are provided a stirring vane 18, a developing roller 13 and a supply roller 17.

The developing roller 13 is provided so as to be partially brought into contact with the photosensitive drum 1 and to be rotatable in the direction B opposite to the rotating direction of the photosensitive drum 1. The supply roller 17 is in contact with the developing roller 13, and rotates in the same direction C as the developing roller 13 so that the toner 19 charged by the stirring vane 18 in a toner vessel 23a and then attached to the outer periphery of the developing roller 17 is fed to the outer periphery of the developing roller 17. As developing methods other than such a mono-component contact developing method, there are known a mono-component non-contact developing method, a two-component contact developing method, and a two-component non-contact developing method.

At a position between the contact point between the developing roller 13 and the supply roller 17 and the contact point between the developing roller 13 and the photosensitive drum 1, there is provided, as a member for regulating the thickness of a toner layer, a blade 15 for the developing roller on the periphery of the developing roller 13. The blade 15 for the developing roller is composed of, for example, a conductive rubber elastic member or a metal.

The transfer step is carried out to transfer a toner image formed on the surface of the photosensitive drum 1 by the developing device 21 onto a recording medium 11 such as paper. Transfer is usually carried out using a transfer roller such as the transfer roller 9 shown in FIG. 2, but belt transfer or corona transfer may also be carried out.

The cleaning step is carried out to clean up the toner remaining on the surface of the photosensitive drum 1. In the case of the image-forming apparatus shown in FIG. 2, a cleaning blade 25 is used. The cleaning blade 25 may be

composed of a rubber elastic member made of, for example, polyurethane, an acrylonitrile-butadiene copolymer or the like.

In the image-forming apparatus shown in FIG. 2, the entire surface of the photosensitive drum 1 is uniformly negatively charged by the charging roller 5, and then an electrostatic latent image is formed by the light irradiation device 7, and then a toner image is formed by the developing device 21. The thus formed toner image on the photosensitive drum 1 is transferred onto a recording medium such as paper, an OHP sheet, another transparent film or the like by the transfer roller 9. The toner not transferred but remaining on the surface of the photosensitive drum 1 is cleaned up by the cleaning blade 25. Then, the next image-forming cycle is started.

The fixing step is carried out to fix the toner image transferred onto the recording medium 11. In the image-forming apparatus shown in FIG. 2, at least one of the heat roller 27a heated by a heating means (not shown) and the support roller 27b is rotated, and therefore the recording medium 11 is heated and pressed when passing between the heat roller 27a and the support roller 27b.

The image-forming apparatus shown in FIG. 2 is designed as a monochrome image-forming apparatus, but the toner of the present invention can also be used in color image-forming apparatuses such as color copying machines and color printers.

## EXAMPLES

Hereinbelow, the present invention will be described in more detail with reference to the following examples. It goes without saying that the scope of the present invention is not limited to these examples. It is to be noted that in the following examples, the terms "part(s)" and "%" refer to "part(s) by weight" and "% by weight", respectively, unless otherwise specified.

### [Evaluation Methods]

Toners of the following examples and comparative examples were evaluated by the methods described below.

#### <Measurement of Physical Properties of Toner>

##### (1) Shape Factor (SF-1, SF-2)

The toner was photographed using an FE-SEM (field emission-type scanning electron microscope, product name: S-4700; manufactured by Hitachi, Ltd.), and then 1000 colored particles were randomly sampled in the micrograph. The image information of these colored particles was analyzed by an image analyzer (product name: Luzex3; manufactured by NIRECO Corporation) to obtain values of SF-1 and SF-2.

##### (2) Viscoelasticity of Toner

The dynamic viscoelasticity of the toner was measured using a dynamic viscoelasticity measuring instrument (rheometer) (product name: RDA-II; manufactured by Rheometrics) at different temperatures while the temperature of the toner was increased at a constant frequency to calculate loss tangents ( $\tan \delta$ ).

Measurement conditions are as follows.

#### <Measurement Conditions>

Measurement tool: A parallel plate having a diameter of 7.9 mm was used for a high-elastic modulus sample and a parallel plate having a diameter of 25 mm was used for a low-elastic modulus sample.

Sample to be measured: A toner molded into a disk-shaped sample having a diameter of about 25 mm and a thickness from 2 to 3 mm

Measurement frequency: 6.28 radian/sec

Measurement strain: Initially set to 0.1%.

Correction for sample elongation: Adjusted by an automatic measurement mode.

Measurement temperature: Increased at a rate of 1° C./min from 30 to 200° C.

##### 5 (3) Observation of Release Agent in Cross-Section of Toner

The toner was dispersed in an epoxy resin, cured, cooled to a temperature of -80° C., and cut with a microtome to prepare a thin slice. The thin slice was stained with a vapor of 0.5% aqueous solution of ruthenium tetroxide for about 5 minutes, and then the stained thin slice was observed with a TEM (transmission electron microscope) (product name: JEM-2500SE; manufactured by JEOL) (magnification:  $\times 5,000$  to  $\times 6,000$ ).

15 The concentration of the toner in a sample obtained by dispersing the toner in an epoxy resin was adjusted so that 5 to 10 cross-sections of the colored particles was observed in a TEM image covering an area of  $28 \times 35 \mu\text{m}$ . Among the colored particles observed in the TEM image covering an area of  $28 \times 35 \mu\text{m}$ , one whose cross-section was not entirely shown and one whose cross-sectional size was not 0.6 to 1.2 times the volume average particle diameter of the colored particle were excluded from evaluation. The cross-sections of the colored particles other than such colored particles excluded from evaluation were observed on the TEM screen to determine the diameters of island-shaped separate phases of the release agent. The average diameter of the island-shaped separate phases was defined as a dispersed diameter of the release agent.

##### 30 (4) Shelf Stability of Toner

20 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 950

19

the printing density after the peeling-off of a tape is defined as ID (after), the fixing rate can be calculated from the following formula:

$$\text{Fixing rate}(\%) = (\text{ID}(\text{after})/\text{ID}(\text{before})) \times 100$$

Here, the tape peeling operation means a series of operation in which a pressure-sensitive adhesive tape (product name: Scotch Mending Tape 810-3-18; manufactured by Sumitomo 3M Limited) is attached to an area to be measured (i.e. a solid pattern printing area) on a test sheet of paper, pressed at a constant pressure to be adhered to the sheet, and peeled off from the test sheet in a direction along the test sheet (i.e. in a direction horizontal to the test sheet) at a constant rate.

The printing density was measured using a reflection image densitometer (product name: RD-914; manufactured by Mcbeth Co.). In this fixing test, the lowest temperature of the fixing roller at which the fixing rate was 80% or higher was defined as the minimum fixing temperature of the toner.

A temperature at which a residual adherent caused by hot offset was observed on the fixing roller whose temperature was increased by 10° C. was defined as a hot offset temperature.

#### (6) Durability (Fog on Photosensitive Member)

Sheets of paper for printing were fed into the modified printer used in the above (5), and the toner was charged into a developing device of the printer. The printer was left in an N/N environment (temperature: 23° C., humidity: 50%) all day long. Then, continuous printing was carried out using the printer at a printing density of 5%, and a printing density and a fog value were measured after printing of every 1,000 sheets.

The printing density was measured in the following manner. Solid pattern printing (i.e. printing at a printing density of 100%) was performed on a sheet of paper, and the printing density of the sheet of paper was measured using a reflection image densitometer (product name: RD-914; manufactured by Macbeth Co.). It is to be noted that in the present invention the term "solid pattern printing" means printing at a printing density of 100%.

The fog value was measured in the following manner. During plain pattern printing (i.e. printing at a printing density of 0%), the operation of the printer was suspended after development. Then, a pressure-sensitive adhesive tape (product name: Scotch Mending Tape 810-3-18; manufactured by Sumitomo 3M Limited) was attached to the photosensitive member to adhere the toner on a non-image part to the tape. The pressure-sensitive adhesive tape was then attached to an unused sheet of paper for printing to measure the color tone thereof using a spectral colorimeter (product name: SE-2000; manufactured by Nippon Denshoku Kogyo K.K.). As a control (i.e. a standard sample), an unused pressure-sensitive adhesive tape was attached to a sheet of paper for printing to measure the color tone thereof in the same manner as described above. These color tones were expressed as coordinates on an L<sub>a</sub>x<sub>b</sub> space, a color difference ΔE was calculated from the color tones of the sample to be measured and the standard sample, and was defined as a fog value. A smaller fog value means less fog, that is, higher image quality. It is to be noted that in the present invention, the term "plain pattern printing" means printing at a printing density of 0%, that is, plain white printing.

A durability test was carried out in the following manner. Printing was continuously performed so long as a printing density as measured when solid pattern printing was performed was 1.3 or higher and the fog value as measured when plain pattern printing was performed was 1% or less, and was

20

stopped when the number of sheets of paper reached 15,000. In the test results, "15,000<" means that the above requirements were satisfied when continuous printing of 15,000 sheets of paper was completed.

#### 5 (7) Cleaning Property

Continuous printing of 15,000 sheets of paper was performed in the same manner as in the above (6), and the photosensitive member and a charging roller were visually observed after printing of every 1,000 sheets of paper to see whether or not the toner escaped a cleaning blade to cause poor cleaning. The cleaning property of the toner was evaluated by the number of sheets of paper printed until poor cleaning was observed (hereinafter, referred to as the "number of sheets printed until poor cleaning occurs")

#### 15 (8) Filming Resistance

Continuous printing of 15,000 sheets of paper was performed in the same manner as in the above (6), and the photosensitive member was visually observed after printing of every 1,000 sheets of paper to see whether or not filming 20 occurred on the photosensitive member. The filming resistance of the toner was evaluated by the number of sheets of paper printed until filming was observed (hereinafter, referred to as the "number of sheets printed until filming occurs").

[Synthesis of Negative Charge Control Resin]

#### Production Example 1

##### Synthesis of Negative Charge Control Resin 1

30 85 parts of styrene, 13 parts of n-butyl acrylate, and 2 parts of 2-acrylamide-2-methylpropanesulfonic acid were added to 900 parts of toluene, and they were reacted in the presence of 4 parts of azobisisdimethyl valeronitrile at 80° C. for 8 hours. After the completion of the reaction, toluene was removed by 35 distillation under a reduced pressure to obtain a sulfonic acid group-containing copolymer. The weight average molecular weight (Mw) of the sulfonic acid group-containing copolymer was 22,000. The thus obtained sulfonic acid group-containing copolymer is hereinafter referred to as a negative charge control resin 1. The amount of a functional group-containing structural unit contained in the negative charge control resin 1 was 2% by weight.

#### Production Example 2

##### Synthesis of Viscoelasticity Control Resin 1

100 parts of an isobornyl acrylate monomer was charged into 900 parts of toluene, and they were heated to 80° C. and 50 reacted for 8 hours in the presence of 4 parts of azobisisdimethyl valeronitrile as a polymerization initiator. After the completion of the reaction, toluene was removed by distillation under a reduced pressure to obtain an isobornyl acrylate polymer (hereinafter, referred to as a "viscoelasticity control 55 resin 1"). The weight average molecular weight (Mw) and Tg of the polymer were 22,000 and 94° C., respectively.

#### Production Example 3

##### Synthesis of Viscoelasticity Control Resin 2

100 parts of a t-butyl methacrylate monomer was charged into 900 parts of toluene, and they were heated to 80° C. and 60 reacted for 8 hours in the presence of 4 parts of azobisisdimethyl valeronitrile as a polymerization initiator. After the completion of the reaction, toluene was removed by distillation under a reduced pressure to obtain a t-butyl methacrylate

21

polymer (hereinafter, referred to as a "viscoelasticity control resin 2"). The weight average molecular weight (Mw) and Tg of the polymer were 19,000 and 107° C., respectively.

## EXAMPLE

## Example 1

80.5 parts of styrene (ST), 19.0 parts of n-butyl acrylate (BA), 0.5 part of divinylbenzene (DVB), 0.5 part of glycidyl methacrylate (GMA), 1.5 parts of t-dodecylmercaptan (TDM), 5 parts of the isobornyl acrylate polymer (viscoelasticity control resin 1) obtained in the Production example 2, and 6 parts of C.I. Pigment Blue 15:3 (manufactured by Clariant K.K.) as a cyan pigment (cyan colorant) were charged into a media type wet grinding machine (product name: PICO MILL; manufactured by Asada Iron Works Co., Ltd.) to perform wet grinding, and then 5 parts of the negative charge control resin obtained in Production example 1 and 5 parts of dipentaerythritol hexamyrystate (DPEHM) (product name: W663; manufactured by NOF Corporation) as a release agent were added and mixed until dissolved to obtain a polymerizable monomer composition.

On the other hand, 11.8 parts of magnesium chloride was dissolved in 250 parts of ion-exchanged water to prepare an aqueous solution of magnesium chloride, and then an aqueous solution prepared by dissolving 6.6 parts of sodium hydroxide in 50 parts of ion-exchanged water was added little by little to the aqueous solution of magnesium chloride under stirring to prepare an aqueous dispersion containing a magnesium hydroxide colloid (i.e. a hardly water-soluble metal hydroxide colloid) as a dispersion stabilizer.

Further, 1 part of methyl methacrylate (i.e. a polymerizable monomer for shell) was mixed with 65 parts of ion-exchanged water, and the mixture was subject to finely-dispersing treatment using an ultrasonic emulsifier to obtain an aqueous dispersion of a polymerizable monomer for shell.

The polymerizable monomer composition was added to the magnesium hydroxide colloidal dispersion, and the resulting mixture was stirred. Then, 6 parts of t-butyl peroxy-isobutyrate (product name: PERBUTYL IB; manufactured by NFO Corporation) was further added thereto as a polymerization initiator, and the resulting mixture was highly sheared and stirred at 15,000 rpm for 30 minutes using an inline type emulsifier (product name: EBARA MILDER; manufactured by Ebara Corporation) to form droplets of the polymerizable monomer composition.

The aqueous dispersion having the droplet of the polymerizable monomer composition dispersed therein was charged into a reaction vessel equipped with a stirring vane, and was heated to 95° C. After the lapse of about 40 minutes, the aqueous dispersion was cooled to 40° C., and was then again highly sheared and stirred at 18,000 rpm for 5 minutes using the inline type emulsifier to subject the droplets to ovalization. Thereafter, the aqueous dispersion was again heated to 95° C.

After a polymerization conversion rate reached almost 100%, a solution prepared by dissolving, in the aqueous dispersion of the polymerizable monomer for shell, 0.5 part of 2,2'-azobis[2-methyl-N-(2-hydroxyethyl)-propionamide] (product name: VA-086; manufactured by Wako Pure Chemical Industries, Ltd.) as a polymerization initiator for the polymerizable monomer for shell was charged into the reaction vessel. Polymerization reaction was continued for 4 hours, and was stopped by cooling the reaction vessel in water to obtain an aqueous dispersion of colored particles.

22

It is to be noted that the polymerization conversion rate was determined in the following manner and calculated by the following equation.

About 2 g of the aqueous dispersion having the droplets of the polymerizable monomer composition dispersed therein was sampled from the reaction vessel in the course of polymerization, placed in an aluminum plate, and precisely weighed. Then, 2 mL of a 5% ethanol solution of hydroquinone was added as a polymerization inhibitor thereto, and the resulting mixture was heated at 150° C. for about 20 minutes in an oven to evaporate moisture and volatile components, and was then cooled to room temperature. The weight of solid matter remaining on the aluminum plate was precisely weighed.

$$\text{Polymerization conversion rate}(\%) = \{(\text{weight of solid matter remaining on aluminum plate after heating}) / (\text{weight of droplets contained in aqueous dispersion sampled})\} \times 100$$

The thus obtained aqueous dispersion of colored particles was adjusted to pH 6.0 by adding 10% dilute sulfuric acid under stirring at room temperature to dissolve magnesium hydroxide, and was then filtered and dewatered. Then, 250 parts of ion-exchanged water having a temperature of 40° C. was added thereto to obtain an aqueous dispersion, and was again filtered and dewatered. Then, 250 parts of methanol was added thereto, stirred for 1 hour, filtered and dewatered. Thus obtained colored particles were dried. In this way, a colored particle having a volume average particle diameter of 6.7 μm was obtained.

To 100 parts of the obtained colored particles, 1 part of silica fine particles whose number average particle diameter of primary particles was 12 nm (product name: R-104; manufactured by Nippon Aerosil) and 0.5 part of silica fine particles whose number average particle diameter of primary particles was 50 nm (product name: HDK-H05TX; manufactured by Clariant K.K.) were added, and the resulting mixture was stirred at 1,400 rpm for 10 minutes using HENSCHEL MIXER (trade name) to prepare a toner.

## Example 2

A toner was prepared in the same manner as in the Example 1 except that the ratio of amounts of styrene, n-butyl acrylate and divinylbenzene (ST/BA/DVB) charged was changed to 80/19/1 and that 0.5 part of GMA was replaced with 0.5 part of 3,4-epoxycyclohexylmethyl methacrylate (CHMM).

## Example 3

A toner was prepared in the same manner as in the Example 1 except that the ratio of amounts of styrene, n-butyl acrylate and divinylbenzene (ST/BA/DVB) charged was changed to 79/19/2, the amount of TDM was changed from 1.5 parts to 2.0 parts, 0.5 part of GMA was replaced with 0.5 part of vinylcyclohexene monoxide-1,2-epoxy-4-vinyl cyclohexane (VCH), and 5 parts of the isobornyl acrylate polymer (i.e. the viscoelasticity control resin 1) obtained in the Production example 2 was replaced with 5 parts of a t-butyl methacrylate polymer (i.e. the viscoelasticity control resin 2 obtained in the Production example 3).

## Comparative Example 1

A toner was prepared in the same manner as in the Example 1 except that the ratio of amounts of styrene, n-butyl acrylate and divinylbenzene (ST/BA/DVB) charged was changed to 90/10/0.2, 0.5 part of GMA was replaced with 0.5 part of a

MMA macromonomer (MMAMM) (product name: AA-6; manufactured by TOAGASEI Co., Ltd.), the amount of DPEHM was changed to 10 parts, and the amount of the isobornyl acrylate polymer (i.e. the viscoelasticity control resin 1) was changed to 2 parts.

#### Comparative Example 2

A toner was prepared in the same manner as in the Example 1 except that the ratio of amounts of styrene, n-butyl acrylate

(divinylbenzene), MMA (methyl methacrylate), CHMM (3,4-epoxycyclohexylmethyl methacrylate), VCH (vinylcyclohexene monoxide-1,2-epoxy-4-vinylcyclohexane), and MMAMM (MMA macromonomer).

\*2: Abbreviations for release agents: DPEHM (dipentaerythritol hexamyrystate), and LUVAX (polyethylene wax).

\*3: Abbreviations for viscoelasticity control resins: PIBA (isobornyl acrylate polymer obtained in the Production example 2, Tg: 94° C.), and t-BMA (t-butyl methacrylate polymer obtained in the Production example 3, Tg: 107° C.).

TABLE 1

|                                                                                                                 | Example 1                    | Example 2                | Example 3                | Comparative Example 1    | Comparative Example 2    | Comparative Example 3    |
|-----------------------------------------------------------------------------------------------------------------|------------------------------|--------------------------|--------------------------|--------------------------|--------------------------|--------------------------|
| Binder resin (weight ratio of feed amount)*1                                                                    | ST/BA/DVB<br>(80.5/19.0/0.5) | ST/BA/DVB<br>(80/19/1)   | ST/BA/DVB<br>(79/19/2)   | ST/BA/DVB<br>(90/10/0.2) | ST/BA/DVB<br>(90/10/0.2) | ST/BA/DVB<br>(90/10/0.2) |
| Monomer added to binder resin                                                                                   | GMA<br>(0.5 parts)           | CHMM<br>(0.5 parts)      | VCH<br>(0.5 parts)       | MMAMM<br>(0.5 parts)     | MMAMM<br>(0.5 parts)     | MMAMM<br>(1.5 parts)     |
| Release agent (feed amount)*2                                                                                   | DPEHM<br>(5 parts)           | DPEHM<br>(5 parts)       | DPEHM<br>(5 parts)       | DPEHM<br>(10 parts)      | LUVAX<br>(2 parts)       | LUVAX<br>(2 parts)       |
| Added resin (feed amount)*3                                                                                     | PIBA<br>(5 parts)            | PIBA<br>(5 parts)        | t-BMA<br>(5 parts)       | PIBA<br>(2 parts)        | PIBA<br>(2 parts)        | —                        |
| Chain transfer agent (feed amount)                                                                              | TDM<br>(1.5 parts)           | TDM<br>(1.5 parts)       | TDM<br>(2.0 parts)       | TDM<br>(1.5 parts)       | TDM<br>(1.5 parts)       | TDM<br>(1.5 parts)       |
| Number of peaks or shoulders of tan δ                                                                           | 2<br>(61° C.,<br>85° C.)     | 2<br>(62° C.,<br>80° C.) | 2<br>(68° C.,<br>90° C.) | 2<br>(54° C.,<br>79° C.) | 2<br>(55° C., 84° C.)    | 1<br>(52° C.)            |
| Tan δ (maximum value in the range from 100 to 200° C.)                                                          | 0.71                         | 0.68                     | 0.76                     | 0.76                     | 1.1                      | 0.8                      |
| Tan δ (minimum value in the range from 100 to 200° C.)                                                          | 0.35                         | 0.28                     | 0.39                     | 0.25                     | 0.35                     | 0.41                     |
| Tan δ (200° C.)/Tan δ (150° C.)                                                                                 | 1.35                         | 1.26                     | 1.41                     | 1.2                      | 1.24                     | 0.9                      |
| Presence or absence of release agent having dispersed diameter larger than 0.1 times the Dv of colored particle | Absent                       | Absent                   | Absent                   | Present                  | Absent                   | Absent                   |
| SF-1                                                                                                            | 150                          | 155                      | 148                      | 115                      | 136                      | 170                      |
| SF-2                                                                                                            | 128                          | 130                      | 131                      | 113                      | 128                      | 155                      |
| Minimum fixing temperature                                                                                      | 120° C.                      | 120° C.                  | 120° C.                  | 140° C.                  | 130° C.                  | 140° C.                  |
| Hot offset temperature                                                                                          | 200° C.                      | 200° C.                  | 190° C.                  | 200° C.                  | 170° C.                  | 200° C.                  |
| Durability (fog on photosensitive member)                                                                       | 15,000<                      | 15,000<                  | 14,000                   | 15,000                   | 15,000<                  | 14,000                   |
| Number of sheets printed until poor cleaning occurs                                                             | 15,000<                      | 15,000<                  | 15,000<                  | 10,000                   | 15,000                   | 15,000<                  |
| Number of sheets printed until filming occurs                                                                   | 15,000<                      | 15,000<                  | 14,000                   | 8,000                    | 10,000                   | 10,000                   |
| Shelf stability                                                                                                 | 0.5 wt %                     | 0.4 wt %                 | 1.2 wt %                 | 3.5 wt %                 | 2.2 wt %                 | 0.3 wt %                 |
| Volume average particle diameter of colored particle(μm)                                                        | 6.2                          | 6.3                      | 6.1                      | 6.1                      | 6.2                      | 6.0                      |
| Dispersed diameter of release agent (μm)                                                                        | 0.15                         | 0.32                     | 0.29                     | 1.5                      | 0.51                     | 0.44                     |

and divinylbenzene (ST/BA/DVB) charged was changed to 90/10/0.2, 0.5 part of GMA was replaced with 0.5 part of MMAMM, 5 parts of DPEHM was replaced with 2 parts of polyethylene wax (product name: LUVAX-1151; manufactured by Nippon Seiro Co., Ltd.), and the amount of the isobornyl acrylate polymer (i.e. the viscoelasticity control resin 1) was changed to 2 parts.

#### Comparative Example 3

A toner was prepared in the same manner as in the Example 1 except that the ratio of amounts of styrene, n-butyl acrylate and divinylbenzene (ST/BA/DVB) charged was changed to 90/10/0.2, 0.5 part of GMA was replaced with 1.5 parts of MMAMM, 5 parts of DPEHM was replaced with 2 parts of polyethylene wax (product name: LUVAX-1151; manufactured by Nippon Seiro Co., Ltd.), and the isobornyl acrylate polymer (i.e. the viscoelasticity control resin 1) was not used. [Results]

The properties of the toners obtained in the above Examples and Comparative examples and the images formed from these toners were evaluated by the methods described above. The evaluation results are shown in table 1.

It is to be noted that abbreviations shown in Table 1 are as follows.

\*1: Abbreviations for binder resins and polymerizable monomers for shell: ST (styrene), BA (butyl acrylate), DVB

#### [Summary of Evaluation Results]

The toners obtained in Examples 1 to 3 had two maximum values of peaks or shoulders of loss tangent (tan δ) in the range from 50 to 120° C., a loss tangent (tan δ) in the range from 100 to 200° C. of 0.8 or less, and a ratio between a loss tangent at 150° C. (i.e. tan δ (150° C.)) and a loss tangent at 200° C. (i.e. tan δ (200° C.)) (tan δ (200° C.)/tan δ (150° C.)) of 1.2 or more. In addition, the dispersed diameter of the release agent contained in each of the toners is 0.1 times or less shorter than the volume average particle diameter of the colored particle contained in the toner, and the shape factors SF-1 and SF-2 of the colored particle are 130≤SF-1≤170 and 110≤SF-2≤150, respectively.

These toners of Examples 1 to 3 had a low minimum fixing temperature and a high hot offset temperature, and were excellent in printing durability, cleaning properties, filming resistance and shelf stability.

On the other hand, the toner obtained in Comparative example 1 had a large dispersed diameter of the release agent contained in the colored particle, and a small SF-1. The toner of Comparative example 1 was excellent in a hot offset temperature as measured in the image quality test, but the minimum fixing temperature thereof was high. In addition, the toner of Comparative example 1 was inferior to the toners of Examples 1 to 3 in all the printing durability, the number of sheets printed until poor cleaning occurs, the number of sheets printed until filming occurs and shelf stability, particu-

## 25

larly in the number of sheets printed until poor cleaning occurs, the number of sheets printed until filming occurs and shelf stability.

The toner obtained in Comparative example 2 had a loss tangent ( $\tan \delta$ ) in the range from 100 to 200° C. of larger than 0.8. In addition, the toner of Comparative example 2 had a high minimum fixing temperature and a lower hot offset temperature as measured in the image quality test than the toners of Examples 1 to 3, and was inferior to the toners of Examples 1 to 3 in the number of sheets printed until poor cleaning occurs, the number of sheets printed until filming occurs and shelf stability.

The toner obtained in Comparative example 3 had only one peak or shoulder of loss tangent ( $\tan \delta$ ) in the range from 50 to 120° C., and a ratio between a loss tangent at 150° C. ( $\tan \delta(150^\circ \text{ C.})$ ) and a loss tangent at 200° C. ( $\tan \delta(200^\circ \text{ C.})$ ) (i.e.  $\tan \delta(200^\circ \text{ C.})/\tan \delta(150^\circ \text{ C.})$ ) of less than 1.2. The toner of Comparative example 3 was excellent in hot offset temperature and shelf stability, but had a high minimum fixing temperature as measured in the image quality test. In addition, the toner of Comparative example 3 was inferior to the toners of Examples 1 to 3 in printing durability and the number of sheets printed until filming occurs, particularly in the number of sheets printed until filming occurs.

## INDUSTRIAL APPLICABILITY

The toner for developing electrostatic image of the present invention can be widely used in electrophotography, electrostatic recording, electrostatic printing, magnetic recording or the like for electrostatic latent image-developing systems, developing methods and image-forming apparatuses for developing latent images having electrostatic properties, such as an electrostatic latent image, a magnetic latent image or the like, to form images such as photographs, pictures, text, symbols or the like. Particularly, the toner of the present invention is suitable for use in a heat-pressure fixing system, method and apparatus such as heat roller fixing or the like.

## 26

The invention claimed is:

1. A toner for developing electrostatic image comprising a colored particle containing a colorant, a binder resin and a release agent, wherein the toner for developing electrostatic image has two or more peaks of loss tangent ( $\tan \delta$ ) in the range from 50° C. to 120° C., a loss tangent  $\tan \delta$  in the range from 100° C. to 120° C. is 0.8 or less, and a dispersed diameter of the release agent is 0.1 times or less shorter than a volume average particle diameter of the colored particle.

2. The toner for developing electrostatic image according to claim 1, wherein a ratio of a loss tangent at 150° C. ( $\tan \delta(150^\circ \text{ C.})$ ) and a loss tangent at 200° C. ( $\tan \delta(200^\circ \text{ C.})$ ) of the toner for developing electrostatic image “ $\tan \delta(200^\circ \text{ C.})/\tan \delta(150^\circ \text{ C.})$ ” is 1.2 or more.

3. The toner for developing electrostatic image according to claim 1, wherein shape factors SF-1 and SF-2 of the colored particle in the toner for developing electrostatic image are  $130 \leq \text{SF-1} \leq 170$  and  $110 \leq \text{SF-2} \leq 150$ .

4. The toner for developing electrostatic image according to claim 1, wherein the toner for developing electrostatic image is produced by a polymerization method.

5. The toner for developing electrostatic image according to claim 1, wherein a volume average particle diameter ( $D_v$ ) of the colored particle is in the range from 4 to 10  $\mu\text{m}$ .

6. The toner for developing electrostatic image according to claim 1, wherein the release agent is a multifunctional ester compound.

7. An image forming method comprising steps of: a developing process to form a visible image with the toner for developing electrostatic image defined by claim 1 on a photosensitive member, a transferring process to form a transferred image by transferring the visible image on a recording medium, and a fixing process to fix the transferred image on the recorded medium.

8. The toner for developing electrostatic image according to claim 1, wherein the toner for developing electrostatic image has two peaks of loss tangent ( $\tan \delta$ ) in the range from 50° C. to 120° C.

\* \* \* \* \*